

## 1

3,222,284

**EMULSION HYDRAULIC FLUID, CONCENTRATE  
AND METHOD OF PREPARING SAME**George R. Cook, Arlington Heights, Ill., assignor, by  
mesne assignments, to Union Oil Company of California,  
Los Angeles, Calif., a corporation of California

No Drawing. Filed Oct. 6, 1961, Ser. No. 143,314

19 Claims. (Cl. 252—75)

This invention relates to new compositions of matter, and more particularly to hydraulic fluid compositions. A specific feature of the invention is the discovery that certain critical relationships exist in the concentrations, types of ingredients, etc., in water-in-oil, emulsion-type hydraulic fluids. Another feature of the invention is the discovery that the ease of emulsibility, the blend stability in concentrated and diluted form, the attainment of suitable viscosities, and the viscosity stability of the diluted emulsion under shear of fire-resistant hydraulic fluids of the water-in-oil emulsion type are directly and critically influenced by the kind, amounts, and ratios of ingredients.

Fire-resistant hydraulic fluids may be pure synthetic materials, such as phosphate esters, mixtures of phosphate esters, or various chlorinated materials, or may be mixtures of water and water-soluble synthetics or water-in-oil emulsions, comprising a second and more recent type of "snuffer" fluids. This latter type, to which this invention relates, offers excellent fire resistance due to the release of a blanket of steam in the presence of high temperature. These emulsion-type fluids offer excellent fire-resistance, acceptable lubricity, corrosion resistance, hydraulic efficiency, adequate film strength, high viscosity index, oxidation stability, good cooling qualities, and compatibility with equipment. As a result, emulsion-type fluids are being used more extensively in systems operating at high temperatures and pressures where fire-resistance is important, such as in the hydraulic machinery in ships at sea, submarines, wind tunnels, mining equipment, missile launching, and in machinery handling hot ingots or molten metals, or operating near sparks, flames, or hot metal surfaces. Some hydraulic systems operate at temperatures as high as 650° F. and pressures as high as 3000 p.s.i. Standardized tests have been developed for fire-resistance, namely, the high-temperature test (pressure-ignition spray test), the hot manifold test, and the pipe-cleaner test under Specification MIL-F-7100. In addition to these criteria, hydraulic fluids must be devoid of toxic effects, must not harm metals or seals, should not foam or cause erosion, and must be compatible with machinery paint.

The development of water-in-oil, emulsion-type hydraulic fluids meeting these severe demands is difficult because these fluids must also be stable in concentrate form, be easily emulsified, and form stable emulsions having suitable viscosities and viscosity stabilities as evaluated by the Vickers pump test. This test was developed by the industry in cooperation with the Bureau of Mines to evaluate the emulsion stability under shear, simulating the conditions imposed in modern hydraulic machinery, particularly for use in mining operations. The operating conditions are 1000 to 2000 p.s.i. at flow rates of at least 2.0 to as high as 8.0 gallons per minute for 1000 hours. These tests may be conducted at pressures as high as 10,000 p.s.i. To pass the Vickers pump test, the hydraulic fluid must not

## 2

break down or permit excess wear of pump parts over the 1000-hour test period. Although no limits on the weight loss to be tolerated have been established, a total weight loss of 0.0300 gm. is considered excellent. Also, the fluid is evaluated for adequate cooling of the system and for uniformity of viscosity throughout the time of the test. Another feature of this invention is the development of an emulsion-type hydraulic fluid which not only meets the general requirements aforesaid, but also passes the Vickers pump test.

Accordingly, a primary object of this invention is to provide fire-resistant hydraulic fluids of the water-in-oil emulsion type.

An object of this invention is to provide fire-resistant hydraulic fluids of the water-in-oil emulsion type which meet the general requirements for hydraulic fluids in addition to qualifying for use at high pressures and/or high temperatures.

Another object of this invention is to provide fire-resistant hydraulic fluids of the water-in-oil emulsion type which exhibit emulsion stability in dilute and concentrated form.

Another object of this invention is to provide fire-resistant hydraulic fluids of the water-in-oil emulsion type which exhibit emulsion stability in diluted form under extreme pressure and shear conditions.

Still a further object of this invention is to provide fire-resistant hydraulic fluids of the water-in-oil emulsion type characterized by their emulsion stability and viscosity stability in diluted form under extreme pressure conditions, as evaluated by the Vickers pump test, in addition to meeting the other requisites for such a fluid.

These and other objects of this invention will be described or become apparent as the specification proceeds.

Many unique problems have been found to be associated with the formulation of water-in-oil emulsions, and concentrates for their preparation, for use as fire-resistant hydraulic fluids. For example, in evaluating and screening a large number of fluids, it was found that the water content (which is all-important in the stability of soluble-oil emulsions of the O/W type) plays no part in the problems of W/O emulsion stability. The use of various mutual solvents or couplers such as diethylene glycol, hexylene glycol, butyl Cellosolve, etc., which are known to be effective stability enhancers in O/W emulsions, offered no solution to the problem in W/O emulsions. Furthermore, various known emulsifiers such as polyoxyethylene derivatives of fatty acids, esters of fatty acids, alkyl aryl sulfonates, and various surfactants, gave satisfactory emulsions with 40% of water, but the emulsions failed the Vickers pump test due to their breakdown. Additives reported to be useful for enhancement of lubricity or anti-wear were evaluated and found to be ineffective or detrimental. By experiments with W/O emulsions, it was determined that the viscosity of the oil in the emulsion had little, if any, effect upon the apparent viscosity of the emulsion. Bright stocks, however, are excluded as the base oil because of their inherently high viscosity. Distillate oils, such as neutral oils, form the best base oil. With a corresponding water content, the substitution of a 2000-vis. neutral for a 100-vis. neutral gave emulsions of practically the same viscosities.

I have found that by combining certain types of petroleum sulfonates in particular proportions with certain metal alkyl dithiophosphates in particular propor-

tions, and combining this mixture at certain over-all concentrations with distillate mineral oils, e.g., with neutral oils, concentrates exhibiting the desired stability, and emulsions therefrom meeting the severe Vickers pump test and other requirements heretofore mentioned, can be obtained. The invention is more particularly described in relation to a number of examples which are to be considered exemplary and not limiting on the scope thereof.

Table I sets forth the composition of this invention in weight percent based on the additives, active ingredients and on a W/O emulsion blend thereof.

Table I

## A. COMPOSITE OF CONCENTRATE BASED ON ADDITIVES

|                                                 | Weight Percent |               |      |
|-------------------------------------------------|----------------|---------------|------|
|                                                 | Low            | Optimum range | High |
| Additive:                                       |                |               |      |
| Commercial alkali metal petrol sulfonate        | 2.50           | 3.45-5.19     | 6.0  |
| Commercial alkaline earth metal alkyl sulfonate | 1.00           | 1.40-3.36     | 4.51 |
| Commercial metal dialkyl dithiophosphate        | 0.49           | 0.92-1.00     | 1.50 |
| Mineral lubricating oil (balance)               |                |               |      |

## B. COMPOSITION OF CONCENTRATE BASED ON ACTIVE INGREDIENTS

| Ingredient:                          |      |           |      |
|--------------------------------------|------|-----------|------|
| Alkali metal petroleum sulfonate     | 1.55 | 2.14-3.22 | 3.72 |
| Alkaline earth metal alkyl sulfonate | 0.45 | 0.63-1.51 | 2.03 |
| Metal dialkyl dithiophosphate        | 0.47 | 0.88-0.95 | 1.43 |
| Mineral lubricating oil (balance)    |      |           |      |

C. COMPOSITION OF W/O EMULSION (60% CONC.+40% H<sub>2</sub>O) OF B

| Ingredient:                          |       |             |       |
|--------------------------------------|-------|-------------|-------|
| Alkali metal petroleum sulfonate     | 0.93  | 1.29-1.93   | 2.23  |
| Alkaline earth metal alkyl sulfonate | 0.27  | 0.37-0.90   | 1.22  |
| Metal dialkyl dithiophosphate        | 0.28  | 0.53-0.57   | 0.86  |
| Mineral lubricating oil (balance)    | 40.00 | 40.00-40.00 | 40.00 |

In Table I, the concentration of the mineral oil has been omitted to avoid the implication that in each part of the table the concentrations appearing one over the other in a column are used to formulate a composition of this invention. Table I is intended to give the range of concentration of each ingredient that can be used in the overall concentrate, for example, the ratio of concentrations in weight percent alkali metal sulfonate to alkaline earth metal sulfonate is broadly between about 1.55/2.03 or .71 to 3.72/.45 or 8.26, and preferably about 3.22/0.63 or 5.27 to 2.14/1.51 or 1.4, and further provided that the total amount of said sulfonates is greater than about 2.77 (2.14+0.63) and less than about 4.73 (3.22+1.51) weight percent. Preferably, the range of the total amount of said sulfonates is about 3.50 to 3.80 with the preferred amount being about 3.65 weight percent.

In making up concentrates using commercially available alkali metal sulfonates and alkaline earth metal sulfonates, as further herein defined, appropriate adjustments in the amount of commercial addend, which generally is obtained as a mineral oil solution, are made to take into account the mineral oil or other diluent that is present. The amounts of such oil or other diluents are taken into account in the mineral oil portion of the compositions. The concentrations of ingredients in all parts of Table I are subject to modification depending on the active ingredients, based upon precise chemical analysis, of the addends used and also upon the amount of water used to make the final W/O emulsion. The amount of metal

alkyl dithiophosphate, on an active ingredient basis, may vary within the low and high or optimum range limits shown provided the above-defined limitations regarding the ratio of sulfonates and total amounts of sulfonates are met. A broader range (based on active ingredients) of about 0.25 to 1.5 weight percent is specified for general service. The dithiophosphate additive may contain small amounts, in the order of 1.0% by wt. of sulfonates, to aid in solubilizing same in mineral oil. Since this changes the total sulfonate content by only about 0.001% by weight at the most, it can be ignored.

The amount of water used to prepare the final W/O emulsion product is subject to some variation. The purpose of the water is to give fire-resistance properties to the product. According to the U.S. Bureau of Mines, between about 38% to 42% by weight of water gives the most consistent and safe fire-resistant qualities, with the optimum being about 40% by weight. These recommended amounts are varied throughout the industry depending on whether the proportions are established on a volume percent or weight percent basis. Generally, a loss of about 5% by weight of water causes a reduction in the fire-resistant qualities of the product. However, for many purposes adequate fire-resistance can be attained through the use of 25% by weight of water, with the balance being the mineral oil concentrate. There is some tendency for the emulsion to burn in a severe electric arc when only 20% by weight of water is present, and at water concentrations above about 45% by weight, there is an increase in the apparent viscosity of the emulsion, causing cavitation in the pumps which results in failure to pass the Vickers pump test. Water concentrations below about 33% by weight do not give adequate fire-resistance for most purposes. Consequently, the water content of the emulsions contemplated by this invention can have values ranging from about 33 to 45% by weight, with the preferred concentration being 33 to 41% by weight.

A preferred embodiment of this invention consists of a fire-resistant hydraulic fluid concentrate having the foregoing proportions comprising sodium petroleum sulfonate, calcium dodecyl benzene sulfonate, zinc dialkyl dithiophosphate, wherein the alkyl group contains 6 to 8 carbon atoms, and a neutral mineral lubricating oil of the MCSR variety.

In order to illustrate the invention, a series of experiments are described wherein a number of experimental emulsions were prepared using different ingredients or addends, different mineral oils, and waters coming from different sources. Initial experiments established that oil-in-water emulsions prepared using the best known commercial sulfonate-type detergents, emulsifiers, and coupling agents with preferred types of oil and distilled water could not pass the Vickers hydraulic pump test because of excessive wear of the pump parts, breakdown of the emulsion, or failure to allow the establishment of the required pumping rates. Some of these oil-in-water emulsions, though stable and meeting the initial viscosity requirements, exhibited a deterioration of viscosity during the tests and almost a complete breakdown at the conclusion of the tests. Examples I to V are illustrative.

## EXAMPLE I

A series of oil-in-water emulsions containing from about 40% to 50% by volume of concentrates and consisting of petroleum sulfonates (9.92% to 12.48% by wt. based on the additives), 1.98% to 2.51% polyethylene glycol esters, assisting agents such as oleic acid, 0.29% to 0.33%, and Mid-Continent solvent refined mineral lubricating oils (19.8% to 36.0%), with distilled water in amounts ranging from about 50.0% to 66.29%, were prepared, tested, and evaluated by means of the Vickers pump test. All of these oil-in-water emulsions failed the Vickers pump tests either because of poor pumping rates, the development of noise and excessive wear in the pump parts, loss of pump pressure, or for other reasons. This

establishes that oil-in-water type emulsions are unsatisfactory for fire-resistant hydraulic-fluid applications.

### EXAMPLE II

A series of water-in-oil emulsions and water dispersions was prepared containing as the emulsifiers such materials as petroleum sulfonates, glyceryl mono-oleate, and such assisting agents as hexylene glycol and high-molecular-weight alcohols, with and without metal dialkyl dithiophosphates, said materials being present in amounts adjusted to give stable water-in-oil emulsions when mixed with from 66% to 71% of MCSR oil and distilled water or with 63 to 84% distilled water. None of these compositions passed the Vickers pump test although the viscosities of the blends and their stabilities were above acceptable limits.

### EXAMPLE III

A water-in-oil emulsion containing 8.0% by wt. of polyethylene glycol 200 monolaurate, 4.0% polyethylene glycol 600 mono-oleate, 66.0% MCSR lubricating oil, and 22.0% distilled water was prepared. The emulsion had a viscosity at 100° F. of 876 SUS. At the conclusion of the Vickers pump test, which had a duration of three hours, the viscosity at 100° F. was 795 SUS and the pumping rate at the start of the test was 2.0 g.p.m. at 1000 p.s.i. This pumping rate dropped to 1.8 g.p.m. at 480 p.s.i. at the conclusion of the test and the required 1000 p.s.i. pressure could not be reached due to pump vibration. This composition failed the Vickers pump test.

#### EXAMPLE IV

A concentrate and water-in-oil emulsion having the following composition in weight percent, on the basis of the commercial additives, were prepared.

| Ingredients                             | Emulsion<br>wt. percent | Concentrate<br>wt. percent |
|-----------------------------------------|-------------------------|----------------------------|
| Polyoxyethylene sorbitan trioleate..... | 1.08                    | 1.80                       |
| Sorbitan partial fatty esters.....      | 2.92                    | 4.87                       |
| Zinc dialkyl dithiophosphate.....       | 0.56                    | 0.93                       |
| 80/100 Finished neutral MCSR oil.....   | 37.37                   | 62.28                      |
| 170/100 Finished neutral MCSR oil.....  | 18.07                   | 30.12                      |
| Water.....                              | 40.00                   |                            |
| <b>Total.....</b>                       | <b>100.00</b>           | <b>100.00</b>              |

In preparing the concentrate, a base oil comprising 1.00% by wt. of the zinc dialkyl dithiophosphate, 66.73% 80/100 F.N., and 32.27% 170/100 F.N. was used. This base oil was 93.33% of the concentrate and 56% of the emulsion. Storage tests indicated this formulation to be highly acceptable as far as the stability of the concentrate and emulsion are concerned, but the emulsion was not sufficiently shear stable to withstand the rigorous action of the Vickers pump test, and the emulsions were unstable after pumping for a short time. This formulation failed the Vickers pump test.

### EXAMPLE V

15 A concentrate and water-in-oil emulsion having the following composition in weight percent, on the basis of the additives used, were prepared.

| Ingredients                       | Emulsion<br>wt. percent | Concentrate<br>wt. percent |
|-----------------------------------|-------------------------|----------------------------|
| Alkyl aryl sulfonate              | 0.75                    | 1.25                       |
| Sorbitan mono-oleate              | 2.97                    | 4.95                       |
| Zinc dialkyl dithiophosphate      | 0.56                    | 0.94                       |
| 80/100 Finished neutral MCSR oil  | 37.56                   | 62.59                      |
| 170/100 Finished neutral MCSR oil | 18.16                   | 30.27                      |
| Water                             | 40.00                   |                            |
| Total                             | 100.00                  | 100.00                     |

In preparing the concentrate, the base oil of Example 35 IV was used and became 93.80% of the concentrate and 56.28% of the emulsion. The concentrate and emulsion were extremely stable but the emulsion failed the Vickers pump test.

Attention was directed to water-in-oil emulsions, and after a series of screening tests and Vickers pump tests, the compositions shown in Table I were established as illustrative of the invention as these compositions meet the stability and performance tests, hereinafter more fully explained, for an FRHF composition.

Table IA

## COMPOSITIONS OF FRHF CONCENTRATES AND EMULSIONS

| Blend No. ....                        | 12          |           |                      |           | 13          |           |                      |           | 14          |           |                      |           |
|---------------------------------------|-------------|-----------|----------------------|-----------|-------------|-----------|----------------------|-----------|-------------|-----------|----------------------|-----------|
|                                       | Concentrate |           | 60%-40% by wt. emul. |           | Concentrate |           | 60%-40% by wt. emul. |           | Concentrate |           | 60%-40% by wt. emul. |           |
|                                       | Addends     | Act. Ing. | Addends              | Act. Ing. | Addends     | Act. Ing. | Addends              | Act. Ing. | Addends     | Act. Ing. | Addends              | Act. Ing. |
| Ingredients:                          |             |           |                      |           |             |           |                      |           |             |           |                      |           |
| Sodium Petroleum Sulfonate (62%)      | 4.00        | 2.48      | 2.40                 | 1.49      | 5.20        | 3.22      | 3.12                 | 1.93      | 3.45        | 2.14      | 2.07                 | 1.28      |
| Ca Dodecylbenzene Sulfonate (45%)     | 2.60        | 1.17      | 1.56                 | 0.70      | 1.40        | 0.63      | 0.84                 | 0.38      | 3.36        | 1.51      | 2.02                 | .91       |
| Zinc Dialkyl Dithiophosphate (95%)    | 0.93        | 0.88      | 0.56                 | 0.53      | 0.93        | 0.88      | 0.56                 | 0.53      | 1.00        | 0.95      | 0.60                 | .57       |
| 80/100 Neutral (Oil No. 1)            | 62.30       | 63.80     | 37.38                | 38.28     |             |           |                      |           |             |           |                      |           |
| 170/100 Neutral (Oil No. 2)           | 30.17       | 31.67     | 18.10                | 19.00     |             |           |                      |           |             |           |                      |           |
| 80/100 Neutral+10% LSWT (Oil No. 14)  |             |           |                      |           | 62.30       | 63.70     | 37.38                | 38.22     |             |           |                      |           |
| 170/100 Neutral+20% LSWT (Oil No. 15) |             |           |                      |           | 30.17       | 31.57     | 18.10                | 18.94     |             |           |                      |           |
| 100 Pale Oil (No. 3)                  |             |           |                      |           |             |           |                      |           | 92.19       | 95.40     | 55.31                | 57.24     |
| B-P Neutral (Oil No. 5)               |             |           |                      |           |             |           |                      |           | (92.19)     | (95.40)   | (55.31)              | (57.24)   |
| Water                                 |             |           | 40.00                | 40.00     |             |           | 40.00                | 40.00     |             |           | 40.00                | 40.00     |

The B-P neutral oil, No. 5, was substituted for the 100 pale oil in the concentrates and emulsions of Blend No. 14, which values are shown in parentheses. Taking into account the amount of ISWT oil in Blend No. 12, and

No. 12 of Table IA, a further comparison was made with two commercially available hydraulic fluids purported to be suitable for use in mining equipment. The results are shown in Table II.

Table II  
COMPARISON OF VICKERS HYDRAULIC PUMP TEST DATA AT 1,000 P.S.I.

| Product                                     | Blend No. 12            |         | FRHF "A"     |         | FRHF "B"     |         |
|---------------------------------------------|-------------------------|---------|--------------|---------|--------------|---------|
|                                             | Table I<br>W/O Emulsion |         | W/O Emulsion |         | W/O Emulsion |         |
| Total pumpage during 1,000 hr. test (gals.) | 128,698                 |         | 113,181      |         | 120,223      |         |
| Total Average Flow Rate (g.p.m.)            | 2.15                    |         | 1.89         |         | 2.00         |         |
| Type of loss                                | Mg.                     | Percent | Mg.          | Percent | Mg.          | Percent |
| Front Bushing                               | 20.7                    | 0.0118  | 33.8         | 0.0189  | 26.1         | 10.0149 |
| Rear Bushing                                | 20.7                    | 0.0119  | 37.1         | 0.0207  | 25.2         | 10.0141 |
| Rotor                                       | 22.0                    | 0.0068  | 11.0         | 0.0034  | 53.0         | 10.0163 |
| Ring                                        | 257.0                   | 0.1165  | 406.0        | 0.1834  | 256.0        | 10.1158 |
| Vanes and Pin                               | 162.8                   | 0.4384  | 803.4        | 2.1138  | 100.0        | 10.2688 |
| Total loss                                  | 483.2                   | 0.0518  | 1,291.3      | 0.1371  | 460.3        | 10.0491 |

<sup>1</sup> These results were subject to question due to the disintegration of a cork float in the safety circuit. The cork was trapped in the filter but could have changed the properties of the fluid to appear more favorable in the pump test.

using a different basis for adjustments due to the oil contents of the addends, results with two additional emulsion compositions or blends, each containing 40% water, 3.12 wt. percent of sodium petroleum sulfonate, 0.84 wt. percent of calcium dodecylbenzene sulfonate and 0.56 wt. percent of zinc dialkyl dithiophosphate, with one containing 37.40% by wt. of 80/100 neutral, 14.46% by wt. 170/100 neutral with 3.60 wt. percent of ISWT oil, and

Referring to Table II the FRHF "A" would be considered borderline and Blend No. 12 is shown to have successfully passed the Vickers pump test.

Since one of the critical factors in formulating fire-resistant hydraulic fluids is the rubber-seal test, the example Blend No. 12 was evaluated in accordance with ASTM D471 Method at 158° F. The results are shown in Table III.

Table III  
RUBBER-SEAL TEST CONDUCTED WITH FIRE-RESISTANT HYDRAULIC FLUID CONCENTRATE AND EMULSION

Rubber Specimens:

1. Chicago Rawhide (Sirvene) Manufacture, Buna N-Type A
2. Vickers Model 104-E-10 Pump Shaft Seal, part No. 188323 (presumably Buna N)

| FRHF type                   | Concentrate (Blend No. 12) |       |       |       | Emulsion (60% Blend No. 12 in H <sub>2</sub> O) |       |       |       |
|-----------------------------|----------------------------|-------|-------|-------|-------------------------------------------------|-------|-------|-------|
|                             | 1                          |       | 2     |       | 1                                               |       | 2     |       |
| Rubber Specimen Number      | Run 1                      | Run 2 | Run 1 | Run 2 | Run 1                                           | Run 2 | Run 1 | Run 2 |
| Durometer (Hardness Value): |                            |       |       |       |                                                 |       |       |       |
| Initial value               | 92                         | 92    |       |       | 92                                              | 92    |       |       |
| After 70 hours              | 92                         | 92    |       |       | 89                                              | 89    |       |       |
| After 168 hours             | 90                         | 92    |       |       | 86                                              | 87    |       |       |
| After 28 days               | 92                         | 92    |       |       | 83                                              | 83    |       |       |
| Thickness (inches):         |                            |       |       |       |                                                 |       |       |       |
| Initial value               | .061                       | .067  |       |       | .065                                            | .062  |       |       |
| After 70 hours              | .061                       | .067  |       |       | .068                                            | .065  |       |       |
| After 168 hours             | .0615                      | .0675 |       |       | .0695                                           | .0665 |       |       |
| After 28 days               | .061                       | .067  |       |       | .0690                                           | .070  |       |       |
| Volume Change (percent):    |                            |       |       |       |                                                 |       |       |       |
| After 70 hours              | 0.1                        | nil   | -0.5  | -7.5  | 9.9                                             | 8.6   | 12.9  | 1.6   |
| After 168 hours             | 0.5                        | nil   | -4.3  | -7.5  | 9.2                                             | 8.9   | 13.5  | 4.7   |
| After 28 days               | 0.4                        | nil   | -3.3  | -14.6 | 8.1                                             | 16.4  | 14.1  | 4.7   |

TEST NOTES:

1. None of the seals showed any tendency to crack when bent back upon itself.
2. Those seals used with the FRHF emulsion were more pliable at end of test period than those tested in the concentrate.
3. No thickness or hardness measurements could be taken on Pump Shaft Seals.

the other containing 33.66% by weight of 80/100 neutral, 14.46% by weight of 170/100 neutral, and 7.36% by wt. ISWT oil, are shown in Table IA and are additional examples of emulsions within the scope of this invention.

In order to obtain a more critical evaluation of Blend 75 p.s.i.g. The results are shown in Table IV.

In order to further establish the unique physical properties of the fire-resistant hydraulic fluids of this invention, Blend No. 12 was further independently evaluated with the Vickers pump test at a higher pressure, namely 1500

Table IV

## HYDRAULIC PUMP TEST AT 1500 P.S.I.G.

Pump Type: Vickers Vane Type, Model 105-C10, Designed flow rate 7.5 to 8.0 g.p.m. (450 to 480 g.p.h.)  
 Sample: 60% (wt.) Blend No. 12 and 40% (wt.) water (a water-in-oil emulsion was formed)

|                                     |        |         |         |         |         |         |         |         |         |       |
|-------------------------------------|--------|---------|---------|---------|---------|---------|---------|---------|---------|-------|
| Test Hours, Cumulative.....         | 0      | 116.5   | 250     | 374     | 510     | 605     | 700     | 800     | 901.5   | 1,013 |
| Test Hours, Periodic.....           | 0      | 116.5   | 138.5   | 124     | 136     | 95      | 95      | 100     | 101.5   | 111.5 |
| Gallongage Pumped, Cumulative.....  | 53,907 | 115,945 | 171,697 | 233,265 | 273,622 | 313,800 | 356,403 | 400,327 | 448,401 |       |
| Gallongage Pumped, Periodic.....    | 53,907 | 62,038  | 55,752  | 61,568  | 40,357  | 40,178  | 42,603  | 43,924  | 48,074  |       |
| Flow Rate (g.p.h.), Cumulative..... | 462.7  | 463.8   | 459.1   | 457.4   | 450.8   | 448.3   | 445.5   | 444.6   | 442.6   |       |
| Flow Rate (g.p.h.), Periodic.....   | 462.7  | 464.6   | 448.8   | 452.7   | 424.8   | 422.9   | 426.0   | 432.8   | 431.2   |       |
| Operating Pressure (p.s.i.g.).....  | 0      | 1,500   | 1,500   | 1,500   | 1,500   | 1,500   | 1,500   | 1,500   | 1,500   | 1,500 |
| Operating Temperature (° F.).....   | 150    | 150     | 150     | 150     | 185     | 185     | 185     | 185     | 185     | 185   |
| Test Data Obtained:                 |        |         |         |         |         |         |         |         |         |       |
| Viscosity at 100° F. (SUS).....     | 349    | 364     | 367     | 355     | 351     | 367     | 409     | 390     | 416     | 398   |
| Viscosity at 150° F. (SUS).....     | 144    | 148     | 146     | 145     | 141     | 148     | 162     | 158     | 170     | 168   |
| Viscosity at 185° F. (SUS).....     |        |         |         |         |         | 89      | 98      | 87      | 96      | 89    |
| Percent Water (by volume).....      | 36.35  | 35.0    | 35.5    | 35.0    | 35.0    | 34.0    | 35.0    | 36.0    | 37.4    | 39    |

Miscellaneous: The following additions of fluid were made—

At 650 hours, 2 qts. concentrate and 4 qts. water.

At 810 hours, 4 qts. concentrate and 4 qts. water.

At 905 hours, 4 qts. concentrate and 4 qts. water.

| Parts                    | Weight (grams) |              |                | Weight Loss (grams)       |                                |                                          | Percent of Lcss<br>From Start to<br>Finish |
|--------------------------|----------------|--------------|----------------|---------------------------|--------------------------------|------------------------------------------|--------------------------------------------|
|                          | Start          | At 510 Hours | At 1,013 Hours | From start to<br>510 hrs. | From 510 hrs.<br>to 1,013 hrs. | From start to<br>finish at 1,013<br>hrs. |                                            |
| Inner Bushing.....       | 183.0372       | 183.0002     | 182.9528       | 0.0370                    | 0.0474                         | 0.0844                                   | 0.0461                                     |
| Outer Bushing.....       | 177.2394       | 177.2094     | 177.1881       | 0.0300                    | 0.0213                         | 0.0513                                   | 0.0289                                     |
| Ring.....                | 182.4314       | 180.5610     | 180.3320       | 1.8704                    | 0.2280                         | 2.0984                                   | 1.1502                                     |
| Rotor.....               | 323.1153       | 322.6431     | 322.4030       | 0.4722                    | 0.2401                         | 0.7122                                   | 0.2205                                     |
| Vanес and Pin.....       | 37.8296        | 37.4766      | 37.1547        | 0.3530                    | 0.3219                         | 0.6749                                   | 1.7841                                     |
| Percent weight loss..... | 903.6529       | 900.8903     | 900.0316       | 2.7626                    | 0.8587                         | 3.6213                                   |                                            |
|                          |                |              |                | 0.305                     | 0.095                          | 0.401                                    |                                            |

Blends 13 and 14 and the two additional blends containing ISWT oil, when similarly tested, pass the Vickers pump test at pressures up to 1500 p.s.i.g., the flammability tests, and the rubber-seal test, and exhibit acceptable stability in concentrate and emulsion form in addition to passing the other requirements for fire-resistant hydraulic fluids.

40 Blend No. 12.

The results shown in Table IV indicate that the compositions of this invention have exceptional properties as evaluated by the Vickers pump test.

Table V gives the results of flammability tests on

Table V

## FLAMMABILITY TESTS CONDUCTED WITH 60% BLEND NO. 12 AND 40% WATER FORMING A WATER-IN-OIL EMULSION

[1. Federal Test Method Standard 352-T, "Effect of Evaporation on Flammability"

(Pipe Cleaner Test)]

Sample: Emulsion taken from Hydraulic Pump Test reservoir at start of test.

| Test No.                | Before Evaporation<br>(cycles) | After 2 hours<br>Evaporation at<br>150° F. (cycles) | After 4 hours<br>Evaporation at<br>150° F. (cycles) |
|-------------------------|--------------------------------|-----------------------------------------------------|-----------------------------------------------------|
| 1.....                  | 30                             | 24                                                  | 24                                                  |
| 2.....                  | 32                             | 27                                                  | 26                                                  |
| 3.....                  | 33                             | 27                                                  | 23                                                  |
| 4.....                  | 31                             | 24                                                  | 26                                                  |
| 5.....                  | 30                             | 24                                                  | 23                                                  |
| Average.....            | 31.2 (Pass)                    | 25.2 (Pass)                                         | 24.4 (Pass)                                         |
| Minimum Acceptable..... | 24                             | 18                                                  | 12                                                  |

Sample: Emulsion taken from Hydraulic Pump Test reservoir after 1,013 hrs. of testing.

|                         |             |             |             |
|-------------------------|-------------|-------------|-------------|
| 1.....                  | 25          | 23          | 25          |
| 2.....                  | 24          | 22          | 23          |
| 3.....                  | 25          | 25          | 25          |
| 4.....                  | 23          | 22          | 22          |
| 5.....                  | 26          | 25          | 24          |
| Average.....            | 24.6 (Pass) | 23.4 (Pass) | 23.8 (Pass) |
| Minimum Acceptable..... | 24          | 18          | 12          |

## [2. U.S. BUREAU OF MINES FLAMMABILITY TEST]

Sample: Emulsion taken from Hydraulic Pump Test reservoir at start of test.  
 Spontaneous Ignition Temperature of Emulsion, 745° F. (600° F. Minimum Required.)  
 Conditions: A spray test at 150 p.s.i. and fluid temperature of 150° F.  
 Results:

|                                 | Distance from Nozzle (inches) |                  |           |
|---------------------------------|-------------------------------|------------------|-----------|
|                                 | 18                            | 24               | 36        |
| Source of Ignition:             |                               |                  |           |
| Open Flame, ignition.....       | None.....                     | None.....        | None..... |
| Open Flame, propagation.....    | do.....                       | do.....          | do.....   |
| Electric Arc, ignition.....     | Very slight.....              | Very slight..... | Do.....   |
| Electric Arc, propagation.....  | None.....                     | None.....        | Do.....   |
| Butane Torch, ignition.....     | Very slight.....              | Very slight..... | Do.....   |
| Butane, Torch, propagation..... | None.....                     | None.....        | Do.....   |

N.b. These tests were also conducted with samples drawn from the hydraulic pump test at approximately 100-hour intervals. The results obtained were essentially the same as those reported herein.

A number of other fire-resistant hydraulic fluid emulsions prepared using the concentrations of ingredients set forth herein also pass the flammability tests shown in Table V.

In evaluating a number of concentrates and emulsions within and outside of the essentially critical limits of added concentration, I found that the concentrates were generally stable and emulsions prepared therefrom, except

In order to establish the essential, critical nature of the proportions of alkali metal petroleum sulfonate and alkaline earth metal sulfonates, a number of compositions 25 using the preferred materials was formulated and tested for emulsion stability under different conditions, that is, one week at 80° F. and two weeks at 140° F. The results are shown in the following Table VI.

Table VI  
 EMULSION STABILITY TESTS USING MCSR OIL

| Blend Number.....                            | Composition Weight Percent Active Ingredients |       |       |       |       |       |       |       |       |       |       |       |
|----------------------------------------------|-----------------------------------------------|-------|-------|-------|-------|-------|-------|-------|-------|-------|-------|-------|
|                                              | 12                                            | 15    | 16    | 17    | 18    | 19    | 20    | 21    | 22    | 23    | 24    | 25    |
| Sod. Petrol Sulf.....                        | 1.49                                          | 1.40  | 1.58  | 1.58  | 1.49  | 1.77  | 2.00  | 2.08  | 1.95  | 2.00  | 2.12  | 2.32  |
| Ca DB Sulf.....                              | 0.70                                          | .77   | .63   | .74   | .81   | .77   | .27   | .22   | .32   | .32   | .35   | .32   |
| Zn Dialkyl dithiophosphate.....              | .53                                           | .53   | .53   | .53   | .53   | .53   | .53   | .53   | .53   | .53   | .53   | .53   |
| Blend of Neutral Oils.....                   | 57.28                                         | 57.30 | 57.26 | 57.15 | 57.17 | 56.93 | 57.20 | 57.17 | 57.20 | 57.15 | 57.00 | 56.73 |
| Water.....                                   | 40.00                                         | 40.00 | 40.00 | 40.00 | 40.00 | 40.00 | 40.00 | 40.00 | 40.00 | 40.00 | 40.00 | 40.00 |
| Emulsion Stability, One week at 80° F.....   | Ex.                                           | Ex.   | B.    | Fail  | B.    | Fail  | B.    | Fail  | B.    | B.    | B.    | Fail  |
| Emulsion Stability, Two weeks at 140° F..... |                                               |       |       |       |       |       |       |       |       |       |       |       |

| Blend Number.....                            | Composition, Weight Percent Active Ingredients |       |       |       |       |       |       |       |       |       |       |       |
|----------------------------------------------|------------------------------------------------|-------|-------|-------|-------|-------|-------|-------|-------|-------|-------|-------|
|                                              | 26                                             | 27    | 28    | 29    | 13    | 30    | 31    | 32    | 33    | 34    | 35    | 36    |
| Sod. Petrol Sulf.....                        | 2.24                                           | 2.25  | 1.88  | 1.91  | 1.93  | 1.82  | 1.71  | 1.60  | 1.57  | 1.49  | 1.34  | 1.38  |
| Ca DB Sulf.....                              | .37                                            | .36   | .32   | .37   | .38   | .46   | .62   | .75   | .70   | .65   | .65   | .78   |
| Zn Dialkyl dithiophosphate.....              | .53                                            | .53   | .53   | .53   | .53   | .53   | .53   | .53   | .53   | .53   | .53   | .53   |
| Blend of Neutral Oils.....                   | 56.86                                          | 56.86 | 57.27 | 57.19 | 57.19 | 57.19 | 57.22 | 57.25 | 57.15 | 57.28 | 57.48 | 57.31 |
| Water.....                                   | 40.00                                          | 40.00 | 40.00 | 40.00 | 40.00 | 40.00 | 40.00 | 40.00 | 40.00 | 40.00 | 40.00 | 40.00 |
| Emulsion Stability, One week at 80° F.....   | B.                                             | Fail  | Ex.   | Ex.   | Ex.   | Ex.   | B.    | B.    | Fail  | Fail  | Fail  | Fail  |
| Emulsion Stability, Two weeks at 140° F..... |                                                |       |       |       |       |       |       |       |       |       |       |       |

Ex.=Excellent. B.=Borderline. Fail=Failure.

those outside the essential limits, satisfactorily passed the Vickers pump test. However, some of the emulsions prepared therefrom were not sufficiently stable for extended periods of time to meet the industry requirements of sufficient stability to be marketed in emulsion form or to withstand periods of storage or shutdown of the hydraulic machinery using the emulsions. I have found that both the type of mineral lubricating oil and the water used in preparing these emulsions has a decided influence on the emulsion stability. It must be kept in mind that many of the emulsions hereinafter evaluated as "unacceptable" are nevertheless useful since they still meet the critical Vickers pump test and the many other critical requirements for a fire-resistant hydraulic fluid.

All of the compositions shown in Table VI are on an active ingredient basis. The blends of neutral oils used in FRHF Blends Nos. 12, 15 and 19 are the same as previously used, that is, 66.73% of 80/100 finished neutral, and 32.27% of 170/100 finished neutral, with 1.00 by wt. of zinc dialkyl dithiophosphate which on an active ingredient basis places 0.53% of the dithiophosphate in each composition. Blends 20 to 29, 13, and 30 to 36 65 contain 10% and 20% ISWT oil. These blends were tested for two weeks at 140° F.

From the table, it is seen that as the amount of alkali metal sulfonate increases in relation to the amount of alkaline earth metal sulfonate, the emulsion stability becomes borderline or unacceptable. 70

In order to further demonstrate the effects of variations of the concentrations of the active ingredients on the emulsion stability, a series of extensive emulsion stability tests were conducted up to 60 days' time, using both distilled water and demineralized water. The results for the former are shown in Table VII.

Accordingly, the compositions of this invention are defined as fire-resistant hydraulic fluids, characterized by meeting the tests herein enumerated, containing, in concentrate form, a major portion of a mineral lubricating oil, preferably of the MCSR variety, between about 1.55 to 3.72 weight percent of an alkali metal petroleum sul-

Table VII  
EMULSION STABILITY TESTS

| Blend Number               | Composition By Weight Percent Active Ingredients |       |       |       |       |       |       |       |       |       |       |
|----------------------------|--------------------------------------------------|-------|-------|-------|-------|-------|-------|-------|-------|-------|-------|
|                            | 37                                               | 38    | 39    | 40    | 41    | 42    | 43    | 44    | 45    | 46    | 47    |
| Sod. Petrol. Sulf.         | 1.81                                             | 1.49  | 1.43  | 1.35  | 1.32  | 1.28  | 1.25  | 1.21  | 1.17  | 1.12  | 1.36  |
| Ca. D.B. Sulf.             | .39                                              | .70   | .76   | .81   | .87   | .91   | .94   | .98   | 1.02  | 1.17  | .93   |
| Zn Dialkyl dithiophosphate | .57                                              | .57   | .57   | .57   | .57   | .57   | .57   | .57   | .57   | .57   | .57   |
| MCSR Oil                   | 57.23                                            | 57.24 | 57.24 | 57.27 | 57.24 | 57.24 | 57.24 | 57.24 | 57.24 | 57.14 | 57.14 |
| Water*                     | 40.00                                            | 40.00 | 40.00 | 40.00 | 40.00 | 40.00 | 40.00 | 40.00 | 40.00 | 40.00 | 40.00 |
| Emulsion Stability Tests:  |                                                  |       |       |       |       |       |       |       |       |       |       |
| 7 days at—                 |                                                  |       |       |       |       |       |       |       |       |       |       |
| 32° F.                     | Ex.                                              | Ex.   | Ex.   | Ex.   | Ex.   | Ex.   | Ex.   | Ex.   | Ex.   | Ex.   | Ex.   |
| 77° F.                     | Acc.                                             | Acc.  | Acc.  | Ex.   | Ex.   | Ex.   | Ex.   | Ex.   | Ex.   | Ex.   | Ex.   |
| 140° F.                    | B.                                               | Acc.  | Acc.  | Ex.   | Ex.   | Ex.   | Acc.  | Acc.  | Acc.  | Acc.  | Ex.   |
| 30 days at—                |                                                  |       |       |       |       |       |       |       |       |       |       |
| 32° F.                     | Ex.                                              | Ex.   | Ex.   | Ex.   | Ex.   | Ex.   | Ex.   | Ex.   | Ex.   | Ex.   | Ex.   |
| 77° F.                     | Acc.                                             | Acc.  | Acc.  | Acc.  | Ex.   | Ex.   | Ex.   | Ex.   | Acc.  | Ex.   | Ex.   |
| 140° F.                    | B.                                               | B.    | B.    | Acc.  | Acc.  | Acc.  | B.    | Fail  | B.    | B.    | Acc.  |
| 60 days at—                |                                                  |       |       |       |       |       |       |       |       |       |       |
| 32° F.                     | Acc.                                             | Acc.  | Ex.   | Ex.   | Ex.   | Ex.   | Ex.   | Ex.   | Ex.   | Ex.   | —     |
| 77° F.                     | B.                                               | B.    | Acc.  | Acc.  | Ex.   | Ex.   | Acc.  | B.    | Fail  | B.    | —     |
| 140° F.                    | B.                                               | B.    | Acc.  | Acc.  | B.    | Fail  | Fail  | Fail  | B.    | B.    | Fail  |

\*Distilled H<sub>2</sub>O: Ex.=excellent. Acc.=acceptable. B=borderline. Fail=failure.

In the compositions set forth in Table VII, the oil, water, and zinc dialkyl dithiophosphate compositions were maintained substantially constant, and variations in the sulfonate contents were studied. From the data, it is apparent that on an active ingredient basis the range of concentrations for the sulfonates falls within the "low" and "high" ranges set forth in part C of Table I. All of the compositions of Table VII pass the Vickers pump test and are highly acceptable FRHF compositions for the intended purpose. Since a prepared emulsion is not likely to be stored longer than 60 days at temperatures above 100° F. or below 32° F., in the main, compositions 40 to 46 meet the general emulsion stability requirements; and such compositions represent additional examples coming within this invention. The import of the data in Table VII is mainly to point up the effect of slight changes in sulfonate ratios as regards the attainment of long-term storage stability. In every instance, even with the emulsions which fail on agitation or use, the emulsion is restored and is suitable for use. Blend No. 47 was prepared at the same sodium sulfonate to calcium sulfonate ratio (on an active ingredient basis) as Blend No. 12, but with a greater quantity of each sulfonate. The stability data on these two blends is identical, but the viscosity of Blend 47 is higher than practical for the invented purpose. An identical series of blends to those reported in Table VII was prepared, using demineralized water, and the stability data for the emulsions therefrom was identical to that shown in Table VII. The use of tap water produces compositions exhibiting reduced levels of emulsion stability, although, as in the case of the demineralized water, the emulsions pass all of the other tests for a fire-resistant hydraulic fluid. Accordingly, Blends Nos. 12-46 all represent examples of compositions coming within the scope of this invention.

The ingredients used in the compositions of this invention are available commercially and well known in the art.

40 ffonate, about 0.45 to 2.03 weight percent of an alkaline earth metal alkaryl sulfonite, and about 0.47 to 1.43 weight percent of a metal dialkyl dithiophosphate. The foregoing concentrates are blended with about 33% to 42% of water. Other ingredients may be incorporated in the compositions of this invention without departing from the spirit thereof. The principal ingredients are hereinafter more fully defined and illustrated.

45 The alkali metal petroleum sulfonates are oil-soluble alkali metal salts of mahogany sulfonates formed from the treatment of petroleum distillates, preferably from Pennsylvania grade oil or naphthenic-base crude, with fuming sulfuric acid, sulfur trioxide, or sulfur trioxide complexes, followed by separation of the green sulfonic acid sludge and neutralization of the acid-treated oil with the appropriate alkali metal base or oxide. The mahogany sulfonates can be extracted from the unreacted oil 50 by treatment with an organic solvent, such as an aqueous alcoholic solution. Upon distillation of the alcoholic solution, as described in U.S. Patent 2,125,305, the alkali metal mahogany sulfonate is recovered. These detergent materials are commonly described as alkali metal petroleum sulfonates, or alkali metal mahogany sulfonates derived from a naphthenic- or paraffin-base crude. They have average molecular weights of about 500 to 550, 55 preferably of about 500 to 530.

60 Examples are sodium mahogany sulfonate, potassium mahogany sulfonate, lithium mahogany sulfonate, cesium mahogany sulfonate, rubidium mahogany sulfonate, and mixtures thereof, having an average molecular weight of about 500 to 550 and derived from naphthenic or Pennsylvania paraffinic crudes. Sodium and potassium petroleum sulfonates are preferred.

65 The analysis of a typical alkali metal petroleum sulfonate, such as was used in Blend No. 12 and identified as sodium petroleum sulfonate (Sheroseope T), a proprietary product of the Bryton Chemical Company, is shown in Table VIII.

Table VIII

## REPRESENTATIVE SODIUM PETROLEUM SULFONATE ASSAY

|                                      |        | Method <sup>1</sup> | Typical Analysis | Controlling |       |
|--------------------------------------|--------|---------------------|------------------|-------------|-------|
|                                      |        |                     |                  | Min.        | Max.  |
| Sodium Sulfonates (wt percent)...    | 59.8   | (D 855).....        | 62.0             | 61          | 63    |
| Mineral Oil (wt percent).....        | 34.4   | (D 855).....        | 32.7             | .....       | ..... |
| Inorganic Salts (wt percent).....    | 0.4    | (D 855).....        | 0.8              | .....       | ..... |
| Water (wt percent).....              | 3.5    | (D 1364).....       | 4.5              | 4.0         | 5.0   |
| Free NaOH (wt percent).....          | 0.01   | (D 855).....        | 0.04             | .....       | ..... |
| Sodium Carboxylate (wt percent)..... | 2.5    | (D 855).....        | 2.500            | 500         | ..... |
| Average Molecular Wt.....            | 513    | (D 855).....        | 1.02             | .....       | ..... |
| Specific Gravity, 60/60° F.....      | 1.0313 | (D 941).....        | .....            | .....       | ..... |
| API Gravity.....                     | 5.7    | (D 287).....        | .....            | .....       | ..... |
| Sulfated Ash (wt percent).....       | 9.2    | (D 874).....        | .....            | .....       | ..... |
| Acid Number.....                     | <0.03  | (D 974).....        | .....            | .....       | ..... |
| Base Number.....                     | 0.93   | (D 664).....        | .....            | .....       | ..... |
| Viscosity at 210° F. (S.U.S.).....   | 2,934  | (D 445-6).....      | .....            | .....       | ..... |
| Pour Point (° F.).....               | +70    | (D 97).....         | .....            | .....       | ..... |
| Weight per gallon (lbs.).....        | 8.590  | (D 287).....        | 8.5              | .....       | ..... |
| Inorganic Salts.....                 | .....  | .....               | .....            | 1.0         | ..... |
| Sodium Carbonate.....                | .....  | .....               | .....            | 0.3         | ..... |

<sup>1</sup> Determined by ASTM method as indicated.<sup>2</sup> Wide range.

The oil-soluble alkaline earth metal alkaryl sulfonates, which are balanced with the alkali metal petroleum sulfonate in accordance with this invention, have the general formula,



where (R) is one or more alkyl, alkaryl or aralkyl groups, *n* having a value of 1 to 5 or more, and the aromatic nucleus may be a single or condensed ring, or a partially hydrogenated ring. R will generally and preferably contain 10 to 14 carbon atoms, and where two R groups are present, the total number of carbon atoms in these substituent groups is from 17 to 36 per sulfonic acid molecule. The average molecular weight of the alkaline earth metal alkaryl sulfonates used herein may be from about 925 to 975 and preferably is about 940 to 970. In this connection, one particular alkaline earth metal alkaryl sulfonate tested, having an average molecular weight of 890, was unsuitable. The preferred alkaline earth metal

Examples of other alkaline earth alkaryl sulfonates are:

Strontium undecylnaphthalene sulfonate  
Calcium undecylbenzene sulfonate  
Calcium dodecylbenzene sulfonate  
Barium dodecylbenzene sulfonate  
Strontium dodecylbenzene sulfonate  
Calcium tridecylbenzene sulfonate  
Barium tridecylnaphthalene sulfonate  
Strontium decylnaphthalene sulfonate  
Calcium tetradearylbenzene sulfonate  
Barium tetradearylbenzene sulfonate  
Strontium tetradecylnaphthalene sulfonate  
Magnesium dodecylbenzene sulfonate  
Magnesium dodecylnaphthalene sulfonate

The analysis of a typical alkaline earth metal sulfonate, such as was used in Blend No. 12 and identified as calcium dodecylbenzene sulfonate ("Bryton Calcium Sulfonate 45"), a proprietary product of the Bryton Chemical Company, is shown in Table IX.

Table IX  
REPRESENTATIVE CALCIUM DODECYL BENZENE SULFONATE ASSAY

|                                                        |        | Method <sup>1</sup> | Typical Properties | Controlling |       |
|--------------------------------------------------------|--------|---------------------|--------------------|-------------|-------|
|                                                        |        |                     |                    | Min.        | Max.  |
| Calcium sulfonates (wt percent).....                   | 43.8   | (D 1216).....       | 45.0               | .....       | ..... |
| Mineral Oil (wt percent).....                          | 53.0   | (D 1216).....       | 53.5               | 43          | 46    |
| Water (wt percent).....                                | 1.0    | (D 1364).....       | Nil                | .....       | ..... |
| Inorganic Salts (wt percent).....                      | 0.9    | (D 1216).....       | Nil                | .....       | 0.5   |
| Basicity as $\text{Ca}(\text{OH})_2$ (wt percent)..... | 1.6    | (D 1216).....       | .....              | .....       | ..... |
| Calcium Carboxylate (wt percent).....                  | 0.1    | (D 1216).....       | .....              | .....       | ..... |
| Average Molecular Wt.....                              | 944    | (D 1216).....       | 950                | 880.0       | ..... |
| Specific Gravity, 60°/60° F.....                       | 0.9554 | (D 941).....        | (?)                | .....       | ..... |
| API Gravity.....                                       | 16.6°  | (D 287).....        | .....              | .....       | ..... |
| Sulfated Ash (wt percent).....                         | 10.2   | (D 874).....        | .....              | .....       | ..... |
| Base Number.....                                       | 24.6   | (D 664).....        | 23.0               | 14.0        | ..... |
| Viscosity at 210° F. (S.U.S.).....                     | 160.1  | (D 445-6).....      | .....              | .....       | ..... |
| Pour Point (° F.).....                                 | +5     | (D 97).....         | .....              | .....       | ..... |
| Weight per gallon (lbs.).....                          | 7.957  | (D 287).....        | 8.0                | .....       | ..... |

<sup>1</sup> Determined by ASTM method as indicated.<sup>2</sup> Close range.

alkaryl sulfonates are calcium and barium dodecylbenzene sulfonates and their mixtures.

Methods of preparing and purifying these alkaline earth metal sulfonates are described in the prior art, e.g., United States Patents 2,760,970, Le Seur: 2,763,615, Faust: 2,839,470, Warren et al.; 2,856,361, Schllicht; 2,861,951, Carlyle; 2,880,173, Honeycutt; 2,883,340, Wasley et al.; 2,902,448, Collins; 2,943,052, Carlyle et al.; and 2,947,694, Cragson.

The heavy-metal salt of an alkyl dithiophosphate used in accordance with this invention is preferably a zinc or cadmium salt of a dialkyl dithiophosphate of the formula:



wherein R is an alkyl radical having from 4 to 10 carbon atoms, and M is zinc or cadmium. Although other tech-

niques are available, in general these substances are prepared by reacting the corresponding aliphatic alcohol with phosphorus pentasulfide to form the esters. The resulting esters are acidic and readily form salts with bases of the metal M, i.e., with the oxides, hydroxides, sulfides, or carbonates. The R-group may be straight-chain, branched-chain, or cycloaliphatic in structure. The metal salts falling within the definition are oil-soluble and are stable components in the concentrates or dilute emulsions. It is preferred that R have 6 to 8 carbon atoms. Examples include

Zinc dihexyl dithiophosphate  
Zinc dioctyl dithiophosphate  
Zinc dinonyl dithiophosphate  
Zinc dibutyl dithiophosphate

Zinc di-t-butyl dithiophosphate  
Zinc di-pentyl dithiophosphate  
Cadmium dibutyl dithiophosphate  
Cadmium dihexyl dithiophosphate  
5 Cadmium dicyclohexyl dithiophosphate  
Cadmium didecyl dithiophosphate

The following Table X gives the chemical and physical characteristics of a typical zinc dialkyl dithiophosphate (namely the proprietary compound identified as Oronite 10 OLOA 262), such as was used in the preferred blend, No. 12. This product has alkyl groups of 6 to 8 carbon atoms, identified as hexyl, heptyl, and octyl groups.

Table XI gives the chemical and physical characteristics of the mineral lubricating oils used in the preferred compositions of this invention, and in other blends that have been prepared and tested.

Table X  
REPRESENTATIVE ZINC DIALKYL DITHIOPHOSPHATE ASSAY

|                                | Typical Value | Deter-mined Values | Specifications | Test Method* |
|--------------------------------|---------------|--------------------|----------------|--------------|
| Phosphorus (wt. percent)       | 7.2           | 7.6                | 6.8-7.6        |              |
| Sulfur (wt. percent)           | 14.75         | 15.6               | 190% of P min. |              |
| Zinc (wt. percent)             | 7.7           | 8.12               | 105 to 115% P  |              |
| Sulfated Ash (wt. percent)     | 25.0          |                    |                |              |
| Vis./100° F. (SUS)             | 485           |                    |                |              |
| Vis./210° F. (SUS)             | 50            | 50.4               |                |              |
| Flash Point (° F.)             | 330           |                    | 320 min        |              |
| Pour Point (° F.)              | -10           |                    |                |              |
| Color                          | 4             |                    |                |              |
| Specific Gravity at 60°/60° F. | 1.08          |                    |                |              |
| Acid No.                       | 130           |                    |                |              |
| Base No.                       | 4.4           |                    |                |              |

\*Determined by ASTM method as indicated.

Table XI  
CHEMICAL AND PHYSICAL CHARACTERISTICS OF MINERAL LUBRICATING OILS

| Oil Identification No.              | Characteristics (ASTM Methods) |                     |             |            |                   |
|-------------------------------------|--------------------------------|---------------------|-------------|------------|-------------------|
|                                     | API Gravity, degs.             | Sp. Gr., 60°/60° F. | Flash, ° F. | Fire, ° F. | Vis./100° F., SUS |
| 1. 80/100 MCSR Neutral              | 35.9                           | 0.8453              | 385         | 420        | 79.7              |
| 2. 170/100 MCSR Neutral             | 31.3                           | 0.8692              | 430         | 480        | 172.3             |
| 3. 100 Pale Oil                     | 22.4                           | 0.9189              | 350         | 410        | 102               |
| 4. 100 Neutral (L)                  | 22.5                           | 0.9188              | 355         | 375        | 105               |
| 5. B-P-Neutral                      | 22.3                           | 0.9195              | 340         | 370        | 109               |
| 6. B-P-Neutral                      | 22.2                           | 0.9201              | 340         | 380        | 113.5             |
| 7. 100 Pale Oil                     | 21.7                           | 0.9236              | 360         | 390        | 103.1             |
| 8. 100 Pale Oil                     | 22.2                           | 0.9206              |             |            | 104.8             |
| 9. 100 Pale Oil                     | 22.4                           | 0.9194              |             |            | 99.7              |
| 10. 100 Pale Oil                    | 22.1                           | 0.9212              |             |            | 104.5             |
| 11. 100 Pale Oil                    | 22.7                           | 0.9176              |             |            | 103.8             |
| 12. 100 Pale Oil                    | 21.8                           | 0.9230              |             |            | 102.9             |
| 13. 100 Pale Oil                    | 21.8                           | 0.9230              |             |            | 102.5             |
| 14. 80/100 MCSR Neut. and 10% ISWT  | 35.6                           | 0.8458              | 360         | 420        | 81.2              |
| 15. 170/100 MCSR Neut. and 20% ISWT | 31.4                           | 0.8686              | 435         | 475        | 175.7             |

| Oil Identification No.              | Characteristics (ASTM Methods) |                    |      |                |                 |                                                             |
|-------------------------------------|--------------------------------|--------------------|------|----------------|-----------------|-------------------------------------------------------------|
|                                     | Vis./120° F. (SUS)             | Vis./210° F. (SUS) | V.I. | Pour Pt., ° F. | Acid No. (1948) | Interfacial Tension at 88° F. oil against water (dynes cm.) |
| 1. 80/100 MCSR Neutral              | 56.0                           | 37.5               | 99   | -10            | <0.03           |                                                             |
| 2. 170/100 MCSR Neutral             | 93.2                           | 44.7               | 99   | 0              | 0.05            |                                                             |
| 3. 100 Pale Oil                     | 62.9                           | 38.1               | 23   | -60            | <0.03           |                                                             |
| 4. 100 Neutral (L)                  | 64.2                           | 38.2               | 39   | -40            | <0.03           |                                                             |
| 5. B-P-Neutral                      | 66.6                           | 38.8               | 18   | -45            |                 |                                                             |
| 6. B-P-Neutral                      | 66.6                           | 38.8               | 14   | -55            | <0.03           |                                                             |
| 7. 100 Pale Oil                     | 61.3                           | 38.1               | 18   | -65            | <0.03           | 35.5                                                        |
| 8. 100 Pale Oil                     |                                | 38.3               | 22   | -55            | <0.03           | 38.4                                                        |
| 9. 100 Pale Oil                     |                                | 38.1               | 28   | -55            | <0.03           | 37.7                                                        |
| 10. 100 Pale Oil                    |                                | 38.3               | 19   | -50            | <0.03           | 38.4                                                        |
| 11. 100 Pale Oil                    |                                | 38.2               | 19   | -50            | <0.03           | 40.3                                                        |
| 12. 100 Pale Oil                    |                                | 38.2               | 21   | -55            | <0.03           | 40.1                                                        |
| 13. 100 Pale Oil                    |                                | 38.1               | 21   | -55            | <0.03           | 41.3                                                        |
| 14. 80/100 MCSR Neut. and 10% ISWT  | 56.7                           | 37.8               | 103  | 0              | <0.03           | 35.3                                                        |
| 15. 170/100 MCSR Neut. and 20% ISWT | 94.9                           | 45.0               | 100  | 0              | <0.03           | 43.3                                                        |

The aniline points of the lubricating oils shown in Table XI vary from about 140° to 150° F., and the oils may contain from about 1.5 to 2.5 wt. percent sulfur. Oils Nos. 3, and 7-13 are products of the Macmillan Oil Company, oil No. 4 is a product of the Lion Oil Company, and oils Nos. 5 and 6 are products of the Berry Asphalt Company.

To illustrate the method of preparation of the FRHF compositions of this invention, the following example is given:

About 165 lbs. of calcium petroleum sulfonate is pre-heated to about 100° F. to facilitate handling, and 4,405 pounds of neutral oil are charged to a clean mixing kettle, agitated and heated to about 150° F. Forty-eight pounds of zinc dialkyl dithiophosphate are added to the heated oil, agitation is continued, and the temperature maintained at 140° to 150° F. The warm calcium petroleum sulfonate is added, and agitation continued with the temperature maintained at 135° to 145° F.; then 165 pounds of sodium petroleum sulfonate are added to the mixture, and agitation is continued for about one hour after the last addition, with the temperature held at 130° to 140° F. Stirring is continued for about one hour, and the temperature is maintained above about 120° F. At this point, samples may be taken for analysis as to base No. (ASTM D-664), which should be within the range of about 0.7 to 1.7, acid No. (ASTM D-974), which should be about 1.00 to 1.4, and sulfated ash (ASTM D-874), which should be in the range of about 0.66 to 0.80. Also, an emulsion can be prepared by mixing 120 grams of concentrate at above about 120° F. with 80 grams of distilled water, with water at room temperature. Acceptable emulsifying properties are evidenced at this point by emulsification with less than 10 minutes of mixing.

Following these analyses and the preparation of stable samples, all of the water, i.e., 3,186 lbs. deionized water or distilled water, is added as rapidly as possible without agitation during the addition of water. At this time, the temperature of the mixture should not be less than 90° F., and not greater than 130° F. The emulsion is then mixed for about 2 hours and cooled as much as possible. The water content (ASTM D-95) in this example is about 37.5 to 39.0% by volume, and the emulsion is stable after one hour at 150° to 160° F.

The following Table XII gives the physical properties of a concentrate containing 3.45% (2.14% by wt. on active ingredient basis) of sodium petroleum sulfonate (Sherope T or Petronate CR), 3.36% (1.51% by weight on active ingredient basis) of calcium dodecylbenzene sulfonate (Bryton Calcium Sulfonate 45), 1.00% zinc dialkyl dithiophosphate (Oronite 262 or Lubrizol 609), and 92.19% neutral oil, which may be Macmillan 100 pale oil, Lion 100 neutral, or Berry Permaseal neutral, and also the properties of the emulsion prepared therefrom.

Table XII

CONCENTRATE (BLEND NO. 37)

| Property                                                                | Sample No. 1 | Sample No. 2 |
|-------------------------------------------------------------------------|--------------|--------------|
| Vis. at 100° F. (SUS)                                                   | 118.6        | 119.1        |
| Vis. at 210° F. (SUS)                                                   | 39.4         | 39.5         |
| H <sub>2</sub> O Content, wt. percent (ASTM D-1364)                     | 0.14         | 0.14         |
| API gravity                                                             | 20.8°        | 20.8°        |
| Sp. Gr. at 60°/60° F.                                                   | .9291        | .9291        |
| Flash Point (° F.)                                                      | 355          | 355          |
| Fire Point (° F.)                                                       | 390          | 390          |
| Aniline Point (° F.)                                                    | 150.0        | 150.7        |
| Pour Point (° F.)                                                       | -50.0        | -55.0        |
| Sulfated Ash (wt. percent)                                              | 0.72         | 0.74         |
| Base No. (ASTM D-664)                                                   | 1.2          | 1.2          |
| Acid No. (ASTM D-664)                                                   | 2.3          | 2.6          |
| Acid No. (ASTM D-974)                                                   | 1.05         | 1.07         |
| Viscosity Index                                                         | 33           | 33           |
| Color (ASTM D-155)                                                      | 3½+          | 3½+          |
| Interfacial Tension at 88° F., oil against H <sub>2</sub> O (dynes/cm.) | 23.7         | 22.9         |

## FIRE-RESISTANT HYDRAULIC-FLUID W/O EMULSION

|    | By Weight                                                                                                                                                 | By Volume                                                      |
|----|-----------------------------------------------------------------------------------------------------------------------------------------------------------|----------------------------------------------------------------|
| 5  | 60%-----<br>40%-----                                                                                                                                      | 61.75% (Blend No. 37).<br>38.25% Distilled or deionized water. |
| 10 | Apparent Viscosity at 100° F. (before use).<br>Apparent Viscosity at 130° F. (before use).<br>Sp. Gr. at 60°/60° F.<br>API Gravity.<br>Weight per gallon. | 423 SUS.<br>217 SUS.<br>0.9567.<br>16.4°.<br>7,967 lbs.        |

The embodiments of this invention in which an exclusive property or privilege is claimed are defined as follows.

1. A hydraulic-fluid concentrate consisting essentially of a major portion of a neutral mineral lubricating oil and the following ingredients:

| Ingredient                                                                                                                                                                                                            | Weight percent |
|-----------------------------------------------------------------------------------------------------------------------------------------------------------------------------------------------------------------------|----------------|
| Alkali metal petroleum sulfonate (mol. wt. about 500-550)                                                                                                                                                             | 1.55 to 3.72   |
| Alkaline earth metal alkylaryl sulfonate (av. mol. wt. about 925-975) containing 10 to 14 carbon atoms in the alkyl portion and said aryl portion being a member of the group consisting of phenylene and naphthylene | 0.45 to 2.03   |
| Metal di-C <sub>4</sub> to C <sub>10</sub> alkyl dithiophosphate wherein the metal is of the group consisting of zinc and cadmium                                                                                     | 0.47 to 1.43   |

wherein the ratio of concentration of alkali metal petroleum sulfonate to alkaline earth metal sulfonate is about 0.71 to 8.26, and the total amount of said sulfonates is greater than about 2.77 weight percent and less than about 4.73 weight percent.

2. A hydraulic-fluid concentrate in accordance with claim 1 in which said alkali metal petroleum sulfonate is sodium petroleum sulfonate.

3. A hydraulic-fluid concentrate in accordance with claim 1 in which said alkaline earth metal alkylaryl sulfonate is calcium dodecylbenzene sulfonate.

4. A hydraulic-fluid concentrate in accordance with claim 1 in which the total amount of said sulfonates is about 3.50 to 3.80 weight percent.

5. A hydraulic-fluid concentrate in accordance with claim 4 in which the total amount of said sulfonates is about 3.65 weight percent.

6. A hydraulic-fluid concentrate consisting essentially of a major portion of a neutral mineral lubricating oil and the following ingredients:

| Ingredient                                                                                                                                                                                                                | Weight percent |
|---------------------------------------------------------------------------------------------------------------------------------------------------------------------------------------------------------------------------|----------------|
| Alkali Metal petroleum sulfonate (mol. wt. about 500-550)                                                                                                                                                                 | 2.14 to 3.22   |
| Alkaline earth metal alkylaryl sulfonate (av. mol. wt. about 925-975) and containing 10 to 14 carbon atoms in the alkyl portion and said aryl portion being a member of the group consisting of phenylene and naphthylene | 0.63 to 1.51   |
| Metal di-C <sub>4</sub> to C <sub>10</sub> alkyl dithiophosphate wherein the metal is of the group consisting of zinc and cadmium                                                                                         | 0.88 to 0.95   |

wherein the ratio of concentration of alkali metal petroleum sulfonate to alkaline earth metal sulfonate is about 0.71 to 8.26, and the total amount of said sulfonates is greater than about 2.77 weight percent and less than about 4.73 weight percent.

7. A hydraulic-fluid concentrate in accordance with claim 6 in which said alkali metal petroleum sulfonate is sodium petroleum sulfonate.

21

8. A hydraulic-fluid concentrate in accordance with claim 6 in which said alkaline earth metal alkylaryl sulfonate is calcium dodecylbenzene sulfonate.

9. A hydraulic-fluid concentrate in accordance with claim 6 in which the total amount of said sulfonates is about 3.50 to 3.80 weight percent.

10. A hydraulic-fluid concentrate in accordance with claim 6 in which the total amount of said sulfonate is about 3.65 weight percent.

11. A hydraulic-fluid concentrate consisting essentially of a major portion of a neutral mineral lubricating oil, about 2.48% by weight of sodium petroleum sulfonate, about 1.17% by weight of calcium dodecylbenzene sulfonate, and about 0.88% by weight of zinc dialkyl dithiophosphate in which the alkyl groups contain 6 to 8 carbon atoms. 10

12. A hydraulic-fluid concentrate consisting essentially of a major portion of a neutral mineral lubricating oil, about 1.93% by weight of sodium petroleum sulfonate, about 0.38% by weight of calcium dodecylbenzene sulfonate, and about 0.53% by weight of zinc dialkyl dithiophosphate in which the alkyl groups contain 6 to 8 carbon atoms. 20

13. A hydraulic-fluid concentrate consisting essentially of a major portion of a neutral mineral lubricating oil, about 2.14% by weight of sodium petroleum sulfonate, about 1.51% by weight of calcium dodecylbenzene sulfonate, and about 0.95% by weight of zinc dialkyl dithiophosphate in which the alkyl groups contain 6 to 8 carbon atoms. 25

14. The method of preparing a hydraulic-fluid concentrate which consists in mixing a neutral mineral lubricating oil with a metal di-C<sub>4</sub> to C<sub>10</sub> alkyl dithiophosphate wherein the metal is of the group consisting of zinc and cadmium at a temperature of about 140° to 150° F., adding an alkali metal petroleum sulfonate having a molecular weight of about 500 to 550 to the mixture while same is maintained at said temperature, adding an alkaline earth metal alkylaryl sulfonate having an average molecular weight of about 925 to 975 and containing 10 to 14 carbon atoms in the alkyl portion and said aryl portion being a member of the group consisting of phenylene and naphthylene to said mixture at a temperature of about 130° to 140° F., stirring said mixture for about one hour at a temperature of about 120° F., and allowing said mixture to cool. 30

15. A fire-resistant hydraulic fluid consisting essentially of an emulsion of about 33 to 45% by weight of a water phase and about 67 to 55% by weight of an oil phase which consists in a major portion of a neutral mineral lubricating oil and the following ingredients:

Ingredient— Weight percent

|                                                                                                                                                                                                                       |              |
|-----------------------------------------------------------------------------------------------------------------------------------------------------------------------------------------------------------------------|--------------|
| Alkali Metal petroleum sulfonate (mol. wt. about 500-550)                                                                                                                                                             | 1.55 to 3.72 |
| Alkaline earth metal alkylaryl sulfonate (av. mol. wt. about 925-975) containing 10 to 14 carbon atoms in the alkyl portion and said aryl portion being a member of the group consisting of phenylene and naphthylene | 0.45 to 2.03 |
| Metal di-C <sub>4</sub> -C <sub>10</sub> alkyl dithiophosphate wherein the metal is of the group consisting of zinc and cadmium                                                                                       | 0.47 to 1.43 |

22

wherein the ratio of concentration of alkali metal petroleum sulfonate to alkaline earth metal sulfonate is about 0.71 to 8.26, and the total amount of said sulfonates is greater than about 2.77 weight percent and less than about 4.73 weight percent. 5

16. A fire-resistant hydraulic fluid consisting essentially of an emulsion of about 33 to 45% by weight of a water phase and about 67 to 55% by weight of an oil phase which consists in a major portion of a neutral mineral lubricating oil and the following ingredients:

| Ingredient—                                                                                                                                                                                                           | Weight percent |
|-----------------------------------------------------------------------------------------------------------------------------------------------------------------------------------------------------------------------|----------------|
| Alkali metal petroleum sulfonate (mol. wt. about 500-550)                                                                                                                                                             | 2.14 to 3.22   |
| Alkaline earth metal alkylaryl sulfonate (av. mol. wt. about 925-975) containing 10 to 14 carbon atoms in the alkyl portion and said aryl portion being a member of the group consisting of phenylene and naphthylene | 0.63 to 1.51   |
| Metal di-C <sub>4</sub> -C <sub>10</sub> alkyl dithiophosphate wherein the metal is of the group consisting of zinc and cadmium                                                                                       | 0.88 to 0.95   |

wherein the ratio of concentration of alkali metal petroleum sulfonate to alkaline earth metal sulfonate is about 0.71 to 8.26, and the total amount of said sulfonates is greater than about 2.77 weight percent and less than about 4.73 weight percent. 25

17. A fire-resistant hydraulic fluid consisting essentially of an emulsion of about 33 to 45% by weight of a water phase and about 67 to 55% by weight of an oil phase which consists in a major portion of a neutral mineral lubricating oil, about 2.48% by weight of sodium petroleum sulfonate, about 1.17% by weight of calcium dodecylbenzene sulfonate, and about 0.88% by weight of zinc dialkyl dithiophosphate in which the alkyl groups contain 6 to 8 carbon atoms. 30

18. A fire-resistant hydraulic fluid consisting essentially of an emulsion of about 33 to 45% by weight of a water phase and about 67 to 55% by weight of an oil phase which consists in a major portion of a neutral mineral lubricating oil, about 1.93% by weight of sodium petroleum sulfonate, about 0.38% by weight of calcium dodecylbenzene sulfonate, and about 0.53% by weight of zinc dialkyl dithiophosphate in which the alkyl groups contain 6 to 8 carbon atoms. 35

19. A fire-resistant hydraulic fluid consisting essentially of an emulsion of about 33 to 45% by weight of a water phase and about 67 to 55% by weight of an oil phase which consists in a major portion of a neutral mineral lubricating oil, about 2.14% by weight of sodium petroleum sulfonate, about 1.51% by weight of calcium dodecylbenzene sulfonate, and about 0.95% by weight of zinc dialkyl dithiophosphate in which the alkyl groups contain 6 to 8 carbon atoms. 40

50

20

55

60

65

#### References Cited by the Examiner

#### UNITED STATES PATENTS

60 2,913,411 11/1959 Schiermeier ----- 252—49.5  
2,961,404 11/1960 Francis ----- 252—75

JULIUS GREENWALD, Primary Examiner.

ALBERT T. MEYERS, Examiner.